



JOHN I. VINTON, OF ALTOONA, PENNSYLVANIA.

*Letters Patent No. 89,187, dated April 20, 1869.*

**IMPROVED COMPOUND FOR FORMING CORES FOR MOULDING IRON, &c.**

*The Schedule referred to in these Letters Patent and making part of the same.*

*To all whom it may concern:*

Be it known that I, JOHN I. VINTON, of Altoona, in the county of Blair, and State of Pennsylvania, have invented a new and improved Core Compound; and I do hereby declare that the following is a full, clear, and exact description thereof, which will enable others skilled in the art to make and use the same.

This invention relates to a new and useful improvement in material for making cores in iron and brass foundries, and for all purposes for which cores are used in forming metal castings; and consists in a compound formed of the ingredients hereinafter named, combined as described.

In the manufacture of cores for foundry purposes heretofore, a large quantity of flour is used, with molasses, sour beer, or similar liquids, in combination with loam or sand. This makes not only an expensive core, but a very unsafe one, unless the ingredients are combined in their exact proportions.

A large percentage of worthless and imperfect castings in foundries is caused by improperly-made cores.

Being practically acquainted with the subject, I have made numerous experiments with various substances, with a view of discovering a compound for cores better suited to the purpose than any heretofore used, and

especially with a view of avoiding the use of flour, molasses, and other expensive ingredients.

In carrying out my invention and forming my core compound, I make use of the following ingredients, in about the proportions named, with the most satisfactory results, viz:

Clean sharp sand, twelve parts.

Common moulding sand, four parts.

Coal dust, two parts.

Horse manure, five parts.

The above ingredients are mixed in a solution of clay, to the proper consistency, when the compound is ready for use. The proportions will, of course, be varied to suit the various sizes and shapes of cores used.

My improved compound can also be applied as a facing for iron castings.

Having thus described my invention,

I claim as new, and desire to secure by Letters Patent—

A core compound, for foundry purposes, composed of the ingredients above named, substantially as described.

Witnesses:

A. McCORMICK,  
S. H. SMITH.

JOHN I. VINTON.